



percent. Preferably, a total of about 0.1 weight percent of the oil composition is preferred. The concentrate will be accordingly multiplied in relation to the detergent.

Usually, the parent dibasic acid will be present in from 0.01 to 0.05 weight percent, while the silyl ester will be present in at least 0.05, preferably 0.075 to 0.29 weight percent.

The lubricating oils which find use are hydrocarbonaceous oils of lubricating viscosity, particularly petroleum oils, which may be naphthenic base, paraffin base, asphaltic base and mixed base lubricating oils. Also, synthetic oils such as polymers of hydrocarbon olefins, alkyl aromatics, etc. may be employed.

The silyl esters of this invention may be prepared by any convenient means. Conveniently, a (trialkyl silyl) amine or di(trialkyl silyl)amine may be combined with the desired dicarboxylic acid and heated at elevated temperatures either neat or in an inert solvent. Reference to the method of preparation of silyl esters may be found in C. Eaborn, "Organic Silicon Compounds," Academic Press, Inc., New York, N.Y., 1960, chapters 9 and 11.

The following example is offered by way of illustration and not by way of limitation.

#### EXAMPLE I

Into a reaction flask was introduced 7 g. of terephthalic acid and 25 cc. of di(trimethyl silyl)amine and the mixture heated under nitrogen for 3 hours. After allowing the mixture to cool, long needle-like crystals formed. The mixture was filtered, the crystals dissolved in hexane, the hexane solution filtered and the hexane distilled off. The residue weighed 11.2 g. An infrared spectrum of the product indicated that the desired di(trimethyl silyl) ester of terephthalic acid had been obtained.

Using a highly hindered polyisobutylene succinimide of tetraethylene pentamine (approximately 2 succinimides per tetraethylene pentamine; the polyisobutylene group being of about 1,000 molecular weight) the silyl ester of terephthalic acid was tested as a corrosion inhibitor in an L-38 strip test. Copper and lead strips are immersed in oil formulations using a 480 neutral oil at a temperature of 340° F. for 20 hours and the weight loss determined at the end of this time. The following table indicates the results obtained.

TABLE I

| Inhibitor  | Wt.<br>percent | Detergent,<br>wt. percent | Cu loss, mg.  |                           |                 |
|------------|----------------|---------------------------|---------------|---------------------------|-----------------|
|            |                |                           | Before<br>KCN | After<br>KCN <sup>1</sup> | Pb loss,<br>mg. |
| Ex. I----- | 0.037          | 9.54                      | 25.3          | 28.2                      | 1,521.5         |
| Ex. I----- | 0.185          | 9.54                      | 18.6          | 26.5                      | 5.1             |
|            |                |                           | 18.4          | 25.9                      | 1.1             |

<sup>1</sup> The strip is washed with dilute potassium cyanide solution (cone. 25 wt. percent in H<sub>2</sub>O) to remove copper salts.

To further test the composition of this invention,

engine tests were performed. An L-38 test using a 1-cylinder CLR engine was carried out for 40 hours at an engine speed of 3,150 r.p.m. The results are reported as the bearing weight loss in milligrams. The first compounded oil (A) prepared had 9.54 weight percent of the detergent described above and 0.022 weight percent of terephthalic acid, the maximum amount which could be solubilized. The second compounded oil (B) added to the first oil, the composition of Example I, in an amount to provide 0.16 weight percent of the lubricating oil composition. For (A) there was a bearing weight loss of 303 mg., while for (B), the loss was only 119 mg.

It is evident from the above results, that the silyl esters are effective corrosion inhibitors in lubricating oil in combination with an ashless amine-containing detergent. Moreover, because of the silyl ester solubility in the lubricating oil, a sufficient amount of the corrosion inhibitor can be maintained in the oil to provide adequate protection in an internal combustion engine.

As will be evident to those skilled in the art, various modifications on this invention can be made or followed, in the light of the foregoing disclosure and discussion, without departing from the spirit or scope of the disclosure or from the scope of the following claims.

What is claimed is:

1. A composition of the formula:



wherein A is lower alkyl of from 1 to 3 carbon atoms, R is lower alkyl from 1 to 8 carbon atoms, n is an integer of from 0 to 1 and the carboxyl groups are separated by at least 3 annular carbon atoms.

2. A composition according to claim 1 wherein A is methyl.

3. A composition according to claim 1 wherein the carboxyl groups are para.

4. A composition according to claim 1 wherein R is tert.-butyl and n is 1.

#### References Cited

##### UNITED STATES PATENTS

- |           |        |                                |
|-----------|--------|--------------------------------|
| 2,707,191 | 4/1955 | Martin et al. -- 260—448.2 R X |
| 2,757,208 | 7/1956 | Burkhard ---- 260—448.2 R X    |

TOBIAS E. LEVOW, Primary Examiner

P. F. SHAVER, Assistant Examiner

U.S. CL. X.R.

252—49.6, 389